

# UNITED STATES PATENT OFFICE.

ARCHIBALD J. SINCLAIR, OF CHICAGO, ILLINOIS, ASSIGNOR TO JAMES F. HILL, OF CHICAGO,  
ILLINOIS.

## PROCESS OF COATING POROUS MATERIAL WITH ASPHALT.

No. 893,391.

Specification of Letters Patent.

Patented July 14, 1908.

Application filed July 16, 1906. Serial No. 326,408.

To all whom it may concern:

Be it known that I, ARCHIBALD J. SINCLAIR, a citizen of the United States, residing at Chicago, in the county of Cook and State of Illinois, have invented a certain new and useful Improvement in Processes for Coating Porous Material with Asphalt, of which the following is a specification.

For many purposes it has long been desired to devise effective means for causing wear resisting compounds containing asphalt, or other bituminous ingredients to adhere to the surface of wood. This has heretofore proved an impossibility owing to the fact that the wood is porous and a considerable quantity of moisture is always retained in the pores, and it is a wellknown fact that hydro-carbons, such as asphalt, cannot be caused to adhere to wood in the presence of moisture. The pores of the wood also contain a considerable quantity of air which adds to the difficulty of causing the asphalt to penetrate the wood in such a manner as to cause a proper adhesion between the two. Various expedients have been devised to overcome the difficulty. The wood surfaces, for instance, have been first painted or brushed with hot compounds containing coal tar, asphalt, rosin and the like; but such hot liquid mixtures fail to obtain such a hold upon the surface of the wood as to enable them to bind thereto the coating of asphalt - containing wear-resisting material subsequently applied. A solution of bituminous materials in a volatile solvent have been tried, but it is found that the solvent cannot carry any material proportion of the bituminous material into the pores of the wood to act as an efficient binder.

I have found that the difficulty may be overcome by applying to the surface of the wood to be coated a bituminous material liquid at the temperatures employed, and by strongly heating the surface of the wood in the presence of the bituminous material in such a manner that as the air and moisture are expelled from the pores of the wood by the heat their place is taken by the liquid bituminous matter. The bituminous material thus obtains a secure hold upon the wood, the surface of the wood being practically penetrated by small filaments of bituminous material. To this preliminary coating of binder or cement the final coating of asphalt con-

taining wear resisting material may be applied.

In carrying out my invention I have the floor, roof, or other wood surface which it is desired to coat with asphalt in as dry a condition as possible. When the wood is as dry as possible under ordinary atmospheric conditions I take any suitable bituminous material, such as gilsonite and residuum oil, and heat the same until it is sufficiently fluid to spread freely with a mop, and while it is in this condition I cover the surface of the wood with a sufficient quantity of the material.

The gilsonite is a well known form of asphalt found in the United States, and the residuum oil is the heavy oil left after the distillation of the lighter constituents of crude petroleum. While the proportions may vary, I prefer to employ 40 per cent of the gilsonite and 60 per cent of the residuum oil. After the surface has been coated with the heated mixture I strongly heat the surface of the wood in the presence of the mixture. This heating is most conveniently done by means of suitable irons heated to a point just below red heat. These irons strongly heat the surface of the wood and cause the moisture in the pores to pass upward in the form of steam. This steam, together with the heated air, also contained in the pores of the wood, passes up in the form of bubbles through the heated mixture covering the surface of the wood. An equivalent portion of the heated mixture passes into the pores of the wood thereby forming little anchors of such material in the wood. I continue this process over the area to which the bituminous mixture has been applied until the bubbles of air and steam cease to arise. The wood is then found to be coated by adhesion with a binder or cement formed of the bituminous mixture, which may be allowed to cool while other portions of the surface to be covered may be treated in a similar manner.

When the wood has been properly coated, as above described, I prepare a wear resisting mixture, one of which, suitable for the purpose, is commonly called "mastic", and in its preferred form ordinarily consists of about 18 per cent of asphalt, about 17 per cent of crushed limestone, and about 65 per cent of good clean sharp hot sand. The

mastic is thoroughly mixed and applied, in the manner commonly known in the art, to any desired thickness. The application of this heated wear resisting coating is sufficient 5 to soften the bituminous binder or cement sufficiently to cause the wear resisting coating and the binder to coalesce. The binder or cement thus securely holds the coating of mastic to the wood.

10 In practice I have found that where wood is treated in the manner described it is impossible to peel the coating from the wood except by splitting off the upper surface of the wood and taking it with the mastic 15 coating.

While various bituminous ingredients might be employed, both in the binder and in the surface coating, I prefer to employ in the binder an ingredient similar to the bituminous content of the wear resisting coating to be applied to the wood. For instance 20 I find gilsonite to be a preferable ingredient of the binder or cement, and while any surface coating containing asphalt or other bituminous material may be applied by means 25 of such a binder, I prefer to employ the gilsonite also in the wear resisting coating as I obtain the best results in this manner.

Wood thus prepared is useful for a variety 30 of purposes where a waterproof wear resisting surface is desired. I consider it, however, especially useful for the floors of refrigerator and cold storage cars in which the conditions are more than usually hard, the 35 excessive vibration combined with the constant presence of moisture rendering it impossible to maintain an asphalt surface properly bound to the wood, by any ordinary process.

40 While I prefer to use as a binder a mixture of a bituminous material, solid at ordinary temperatures, and a bituminous oil, liquid at ordinary temperatures, the resulting mixture being also solid at ordinary temperatures, I have obtained a measure of success 45 by using gilsonite only as the binder. Other bituminous materials might be employed, the main condition being that they be liquid at the temperatures employed in the process 50 of heating the surface of the wood, as already described. Although this process is particularly adapted for use when wood is the base to which the wear resisting surface is to be applied, I desire it to be understood 55 that it may equally as well be applied to any other porous materials of a similar nature to wood which contain air and moisture in their pores.

What I claim as my invention is:—

60 1. In a method of causing a coating containing a bituminous ingredient to adhere to the surface of wood, the coating of the surface with a binder or cement containing a bituminous material, and the subsequent heating 65 of the surface in the presence of the ce-

ment to cause the expulsion of air and moisture from the pores of the wood and their replacement by the cement.

2. In a method of causing a coating containing a bituminous ingredient to adhere to the surface of wood, the coating of the surface with a binder or cement containing a bituminous material similar to the bituminous content of the coating to be applied, and the subsequent heating of the surface in the presence of the cement to cause the expulsion of air and moisture from the pores of the wood and their replacement by the cement. 70 75

3. In a method of causing a coating containing a bituminous ingredient to adhere to the surface of wood, the coating of the surface with a binder or cement solid at ordinary temperatures but heated sufficiently to spread freely over the surface, and the subsequent heating of the surface in the presence 80 of the cement to cause the expulsion of air and moisture from the pores of the wood and their replacement by the cement. 85

4. In a method of causing a coating containing a bituminous ingredient to adhere to the surface of wood, the coating of the surface with a cement or binder comprising a mixture of residuum oil and asphalt solid at ordinary temperatures, and the subsequent heating of the surface in the presence of the 90 cement to cause the expulsion of air and moisture from the pores of the wood and their replacement by the cement. 95

5. In a method of causing a coating containing a bituminous ingredient to adhere to the surface of wood, the coating of the surface with a cement or binder comprising a mixture of residuum oil and gilsonite solid at ordinary temperatures, and the subsequent heating of the surface in the presence of the 100 cement to cause the expulsion of air and moisture from the pores of the wood and their replacement by the cement. 105

6. The process of coating wood which consists in a method of causing a coating containing a bituminous ingredient to adhere to the surface of wood, the coating of the surface with a binder or cement containing a bituminous material, the subsequent heating of the surface in the presence of the cement 110 to cause the expulsion of air and moisture from the pores and their replacement by the cement, and the subsequent application to the binder coated surface of a heated wear resisting coating containing a bituminous ingredient. 115 120

7. The process of coating wood which consists in a method of causing a coating containing a bituminous ingredient to adhere to the surface of wood, the coating of the surface with a binder or cement containing a bituminous material similar to the bituminous content of the coating to be applied; the subsequent heating of the surface in the presence of the cement to cause the expulsion of 125 130

air and moisture from the pores and their replacement by the cement, and the subsequent application to the binder coated surface of a heated wear resisting coating containing a bituminous ingredient.

8. The process of coating wood which consists in a method of causing a coating containing a bituminous ingredient to adhere to the surface of wood, the coating of the surface with a cement or binder comprising a mixture of residuum oil and asphalt solid at ordinary temperatures, the subsequent heating of the surface in the presence of the cement to cause the expulsion of air and moisture from the pores of the wood and their replacement by the cement, and the subsequent application to the binder coated surface of a heated wear resisting coating containing a bituminous ingredient.

9. The process of coating wood which con-

sists in a method of causing a coating containing a bituminous ingredient to adhere to the surface of wood, the coating of the surface with a cement or binder comprising a mixture of residuum oil and gilsonite solid 25 at ordinary temperatures, the subsequent heating of the surface in the presence of the cement to cause the expulsion of air and moisture from the pores of the wood and their replacement by the cement, and the 30 subsequent application to the binder coated surface of a heated wear resisting coating containing a bituminous ingredient.

In witness whereof, I have hereunto subscribed my name in the presence of two wit- 35 nesses.

ARCHIBALD J. SINCLAIR.

Witnesses:

HENRY RAMSTRON,  
DWIGHT B. CHEEVER.